

# UNITED STATES PATENT OFFICE.

OLIVER B. McMILLIN, OF PITTSBURGH, PENNSYLVANIA, ASSIGNOR TO PITTSBURGH ROLLS CORPORATION, A CORPORATION OF VIRGINIA.

## METHOD OF MANUFACTURING ROLLS.

1,296,200.

Specification of Letters Patent.

Patented Mar. 4, 1919.

No Drawing.

Application filed March 6, 1918. Serial No. 220,810.

To all whom it may concern:

Be it known that I, OLIVER B. McMILLIN, a citizen of the United States, residing at Pittsburgh, in the county of Allegheny and State of Pennsylvania, have invented certain new and useful Improvements in Methods of Manufacturing Rolls, of which the following is a specification.

My invention consists of an improvement in the manufacture of rolls for rolling mills, and is particularly applicable to the making of "chilled" rolls.

Heretofore, such rolls have ordinarily been made from metal melted in a cupola or air furnace, in either type of which the control of the elements forming the melt is more or less uncertain, and especially as to the sulfur and carbon content, because of the fuel employed and the inability to control the supply of fuel and its consistency. In the making of chilled rolls, it is desirable that the carbon content of the roll at its wearing face, and for a considerable depth inwardly therefrom, shall be in combined form. Also that the range of carbon shall be within 2.76% to 2.95% for best results. In rolls of large section the carbon should be in combined form at least co-extensive with the depth of the chill, and preferably somewhat beyond such depth toward the center. Also that the change from combined carbon to graphitic carbon shall not be abrupt, but gradual, and merging the one into the other. In chilled rolls it is also very desirable to have all other portions except the working face of the roll where strength is required, of a composition in which the carbon is in graphitic form.

Likewise, in the making of chilled rolls, their intended use as finishing rolls and during the last passes of plates, rails, etc., wherein the smallest percentage of reduction is accomplished in the latter passes of the metal through the rolls, it is desirable in a roll of the usual or ordinary gray iron mixture, to pretty accurately control the proportion of sulfur. The control of the silicon, and when used, manganese, is also a matter of importance. These various ingredients, and especially sulfur, are particularly sensitive and affected by the quality and kind of the fuel employed, its volume, the relative proportion of air, and the constant maintenance of the ideal proportions. The carbon

content also is especially effected by these influences. 55

Because of the quality and kind of the fuel used and the uncertainty as to its control and active effect on the contents of the cupola or ordinary air furnace, the results in the mixture in such forms of furnaces, as ordinarily heretofore used in the making of commercial chilled rolls, have been and necessarily are more or less uncertain. This results in a considerable variation in the chemical consistency and content of the casting, in contrast with the desired analysis, and in marked variation from the analysis of the batch as originally made up. The lack of control in a cupola or air furnace 70 frequently results in heavy losses to the manufacturer because of returned or scrapped rolls in which the depth of chill is either too deep or too shallow, due to undesirable variation in some of the essential elements. 75 This is especially true as to sulfur and carbon.

Thus, an original mixture or charge of metal, made up with the purpose of producing a casting having the same corresponding chemical content, may vary widely therefrom, as illustrated in the following formula. The batch as made up, for instance, for good intended results in a gray iron chilled casting would consist of a mixture 80 having the following typical analysis:—

Silicon .60%; sulfur .061%; phosphorus .42%; manganese .26%; total carbon 2.94%; with the balance of the 100% iron.

In changing this formula, as in carbon or 90 sulfur, or in other sensitive elements, I have found that I can control the result in an open hearth furnace so as to maintain the proportions very closely to the desired analysis. 95

Such batch, however, when melted in a cupola or air furnace, may show variations as indicated in the following formula, in the finished chilled roll product:—

Silicon .75%; sulfur .08-1.00%; phosphorus .43%; manganese .15% to .28%; total carbon 2.70% to 3.20%. 100

As to the phosphorus, it is possible to maintain this element in a cupola or air furnace at about the same desirable percentage as originally intended. 105

However, the sulfur is largely increased due to the presence of free sulfur in the coke

in the cupola furnace, or in the coal used in the air furnace.

In either a cupola or air furnace the control or regulations of the supply is always 5 more or less uncertain.

After considerable experimentation and numerous tests, in connection with special and careful manipulation, I have found that with a regenerative open hearth furnace of

10 the Siemens type, or similar construction, I am able to so control the volume and proportions of the fuel, preferably natural gas, as to accurately control the heat, time of melt, oxidation, and the various other necessary elements having a direct effect on the product as produced in the resulting casting, especially when cast in a chill mold, so that the resulting analysis is substantially or exactly the same in the resulting roll as that desired and as indicated, for instance, in the first above noted preferred analysis. This is especially true as to the sulfur and carbon content, and the carbon, as stated, will take the combined form throughout the depth of 20 the chill or at the working portions of the resulting roll.

While I am, of course, aware that open hearth furnaces of the regenerative type have been used for the making of various 30 castings, and that the advantages in some of the respects noted, are well known, I believe that I am the first to have utilized an open hearth furnace in the particular and somewhat technical and special art of manufacturing chilled rolls, having the chemical elements combined in substantially the desired proportions indicated.

The results in practice have shown definite 40 advantages, increased strength and wearing qualities, and greater endurance in high carbon gray iron chilled rolls over anything heretofore produced in this class of rolls.

The practice is in marked contrast to that heretofore commonly followed, utilized and adhered to by makers of this kind of rolls, and the results in use, because of maintaining the integrity of the original analysis, have shown a marked degree of superiority 45 over similar rolls heretofore manufactured and used.

What I claim and desire to secure by Letters Patent is:—

1. The method of making chilled rolls, consisting in forming a mixture of iron containing silicon, sulfur, phosphorus, manganese, and carbon in predetermined proportions, the manganese being low; melting the mixture in an open hearth furnace while maintaining control and avoiding undesirable variations in proportions of said elements; and casting the molten metal while in such controlled condition in a chill mold, substantially as set forth.

2. The method of making chilled rolls, 60 consisting in forming a mixture of iron con-

taining silicon, sulfur, phosphorus, manganese, and carbon in predetermined proportions, the manganese being low; melting the mixture in an open hearth furnace while maintaining control and avoiding undesirable variations in proportions of the sulfur and carbon; and casting the molten metal while in such controlled condition in a chill mold, substantially as set forth.

3. The method of making chilled rolls, 75 consisting in forming a mixture of iron containing silicon, sulfur, phosphorus, manganese, and carbon in predetermined proportions, the manganese being low; melting the mixture in an open hearth furnace while 80 maintaining control and avoiding undesirable variations in proportions of the sulfur and carbon; and casting the molten metal while in such controlled condition in a chill mold, whereby to form a chilled roll in 85 which the carbon content at its face and for a limited distance inwardly thereof is in combined form, substantially as set forth.

4. The method of making chilled rolls, 90 consisting in forming a mixture of iron containing silicon, sulfur, phosphorus, manganese and carbon in predetermined proportions, the manganese being low; melting the mixture in an open hearth furnace while 95 maintaining control and avoiding undesirable variations in proportions of the sulfur and carbon; and casting the molten metal while in such controlled condition in a chill mold, whereby to form a chilled roll in 100 which the carbon content is in combined form co-extensive with the depth of the chill, substantially as set forth.

5. The method of making chilled rolls, 105 consisting in forming a mixture of iron containing silicon, sulfur, phosphorus, manganese and carbon in predetermined proportions; melting the mixture in an open hearth furnace while maintaining control and avoiding undesirable variations in proportions of the sulfur and carbon; and casting the molten metal while in such controlled condition in a chill mold, whereby to form a chilled roll in which the carbon content is in 110 combined form co-extensive with the depth of the chill, and is in graphitic form throughout the central body portion of the roll, substantially as set forth.

6. A chilled roll formed of a mixture of iron having predetermined and controlled proportions of silicon, sulfur, phosphorus, manganese and carbon with the carbon of the outer chilled face portion of the roll in 120 combined form.

7. A chilled roll formed of a mixture of iron having predetermined and controlled 125 proportions of silicon, sulfur, phosphorus, manganese and carbon with the carbon of the outer chilled face portion of the roll in combined form and the carbon of the inner body portion of the roll in graphitic form. 130

8. A chilled roll formed of a mixture of iron having contained proportioned elements as follows: silicon .60%, sulfur .061%, phosphorus .42%, manganese .26%, total carbon 2.94% and with the carbon of the outer chilled face portion of the roll in combined form and with the carbon of the outer chilled face portion of the roll in combined form.

9. A chilled roll formed of a mixture of iron having contained proportioned elements

as follows: silicon .60%, sulfur .061%, phosphorus .42%, manganese .26%, total carbon 2.94% and with the carbon of the outer chilled face portion of the roll in combined form and of the inner body portion in graphitic form.

In testimony whereof I hereunto affix my signature.

OLIVER B. McMILLIN.

Copies of this patent may be obtained for five cents each, by addressing the "Commissioner of Patents, Washington, D. C."